

Patented Apr. 18, 1944

2,347,152

# UNITED STATES PATENT OFFICE

2,347,152

## COMPOUNDED OIL

Elmali W. Gardiner and George H. Denison, Jr.,  
Berkeley, Calif., assignors to Standard Oil Company  
of California, San Francisco, Calif., a corporation  
of Delaware

No Drawing. Application January 13, 1941,  
Serial No. 374,250

11 Claims. (CL 252—54)

This invention relates to a new and useful composition of matter and involves a composition comprising a hydrocarbon oil and a metal phenate of a relatively high molecular weight phenol.

This application is a continuation-in-part of our parent application Serial No. 233,328, filed October 4, 1938, and is directed to a divisional aspect of the invention disclosed in the parent case.

The production of improved hydrocarbon oils, and particularly of lubricating oils having desired characteristics, has been the subject of extensive research and investigation in recent years. Generally speaking, the compounding of hydrocarbon oils to obtain desired characteristics involves empirical phenomena, and the action of untested types of compounding agents cannot be predicted.

A characteristic which has been the subject of extensive investigation is the tendency of hydrocarbon oils to deteriorate or partially decompose when subjected to high temperatures. This deterioration is evidenced by the deposition of adhesive deposits on hot metallic surfaces over which the hydrocarbon oil may flow. It is important that resistance to such deterioration be imparted to hydrocarbon oils, particularly to lubricating oils, in order that such compositions may be relatively free from the tendency to form such deposits even under high temperatures and severe operating conditions. A direct result of this type of deterioration during lubrication of internal combustion engines, such as engines of the Diesel type, is the tendency of the oil to cause or permit the sticking of piston rings. Compounds which render hydrocarbon oils more resistant to deterioration by heat at high temperature levels usually, though not always, impart to the oil the ability to inhibit piston ring sticking in internal combustion engines and permit longer periods of operation of such engines without the necessity of major overhauls heretofore occasioned by stuck piston rings.

It has been discovered that dispersion of metal phenates in hydrocarbon oils, such as mineral lubricating oil, imparts new and unpredictable properties to the composition. These new properties render the compounded oil particularly useful for various purposes. For example, alkaline earth phenates like calcium lauryl phenate, calcium cetyl phenate, barium cetyl phenate, calcium di-amyl phenate, calcium heptyl phenate and other metal phenates like aluminum alkyl phenates and alkali metal alkyl phenates impart to hydrocarbon compositions an increased resistance to deterioration by heat and the ability to inhibit piston ring sticking when used as a crankcase lubricant in internal combustion engines, such as Diesel engines.

In general, it has been discovered that the new compositions herein disclosed are more stable to heat than is the hydrocarbon oil from which the compositions are compounded. The new compositions of this invention are therefore useful wherever resistance to heat is important. An addi-

tional example of such utility comprises use as a heat transfer fluid where it may be desirable to inhibit or prevent the formation of a deposit on the metal surface from or to which heat is being conveyed.

We have also discovered that certain metal phenates have a combination of properties heretofore unknown and particularly desirable in a compounded mineral oil, namely, the ability to 10 impart resistance to deterioration by heat or the ability to inhibit piston ring sticking, freedom from the production of increased wear on cylinder walls and piston rings as compared with un compounded mineral oils, and low corrosivity as respects the chemical action of the compounded oil 15 on bearing metals, such as cadmium-silver alloys. Although various compounded mineral oils are known which are capable of inhibiting piston ring sticking, the discovery of specific compounding agents capable of imparting the above combination 20 of properties to hydrocarbon oils represents an unobvious and important discovery.

Metal phenates which may be added to hydrocarbon oils such as mineral lubricating oils to provide a new composition of matter of the type herein involved comprise the alkali, alkaline earth and other metal phenates. Specific examples of such metal phenates are: sodium phenates, potassium phenates, beryllium phenates, calcium phenates, strontium phenates, barium phenates, 25 magnesium phenates, zinc phenates, cadmium phenates and aluminum phenates.

The phenates are preferably formed from high molecular weight phenols of the type formula:

35



40

in which *u*, *v*, *w*, *x* and *y* are selected from the group consisting of hydrogen, hydrocarbon, oxy and hydroxyl radicals. The phenol preferably contains at least one alkyl group containing more 45 than four carbon atoms. However, it is to be understood that the broader aspects of the invention include other phenols which contain more than ten carbon atoms. The term "hydrocarbon radical" is intended to include alkyl, aryl, aralkyl, 50 alkaryl or cyclic nonbenzenoid groups. The term "oxy radical" refers to a group in which the hydrogen of an hydroxyl radical has been replaced by esterification, neutralization or the like. Although phenols containing at least one alkyl substituent are preferred, the invention does not preclude compounds containing no alkyl groups and embodies the substitution of aryl, alkaryl, aralkyl 55 and cyclic nonbenzenoid groups in the aromatic nucleus to which the phenolic hydroxyl group is directly attached.

Examples of specific compounds which may be utilized comprise sodium lauryl phenate, sodium

cetyl phenate, calcium lauryl phenate, calcium cetyl phenate, calcium diethyl phenate, calcium heptyl phenate, calcium p-tertiary-amyl phenate, calcium mono-chloro-amyl phenate, calcium p-cyclohexyl phenate, aluminum lauryl phenate, aluminum dicetyl phenate, magnesium cetyl phenate, barium cetyl phenate, and calcium cetyl cresylate. These compounds are sufficiently soluble in mineral lubricating oils that they may be added thereto with advantage, as herein previously pointed out.

To guide those skilled in the art in the preparation of the compositions of this invention, the following specific examples are given:

An alkyl phenol desirable for present purposes may be prepared as follows:

*Example 1.*—Phenol and a butene polymer having an apparent molecular weight of 194 and obtained by polymerization of a mixture of butenes containing butene-1, butene-2, and isobutene were mixed. To this mixture, containing 237 grams of phenol and 500 grams of the above-mentioned butene polymers, 140 cubic centimeters of 94% sulfuric acid was added slowly with agitation. The temperature was kept below 65° F. during addition of the acid. The mixture was agitated for two hours after the addition of acid was completed and permitted to come to room temperature. The reaction product was then diluted with an equal volume of water and placed in a sealed autoclave where it was heated at 350° F. for an hour with agitation. The product was washed with water, 5% sodium carbonate solution and again with water in order to free it of sulfuric acid, sulfonates and unreacted phenol. A 93% yield of high molecular weight water-insoluble alkyl phenol having an acetyl number of 181 was obtained.

An additional example of a method of preparing alkyl phenols suitable for use in this invention comprises:

*Example 2.*—511 grams of crude cresylic acid, 900 grams of olefin polymers containing an average of 14 carbon atoms per molecule, and 475 grams of 98% sulfuric acid were utilized in preparing an alkylated cresol. These ingredients were combined and treated in the manner described above for preparation of cetyl phenol. The product was vacuum-distilled at 10 mm. and a 50 to 90% cut of an alkyl phenol obtained which had a molecular weight of 291 and was used to prepare the calcium salt hereinafter described in Example 6.

It is to be understood that the above examples are given by way of illustration only and that other condensation reactions utilizing alcohols, alkyl chlorides and the like rather than olefins may be adopted as a starting material for introducing the alkyl group into the aromatic nucleus. Also, other known condensation agents, such as aluminum chloride, zinc chloride, etc., may be utilized for effecting alkylation of the phenol. A mixture of sulfuric and glacial acetic acids may be used with advantage as a condensing agent. A suitable mixture comprises 100 parts by weight 98%  $H_2SO_4$  to 60 parts by weight of glacial acetic acid. The presence of the acetic acid facilitates temperature control and gives a softer, easier handled reaction product.

The following comprise illustrative examples of methods of preparing the metal phenates of this invention from the alkyl phenols:

*Example 3.*—247 grams of an alkylated phenol having an apparent molecular weight of 247 were

agitated for six hours at 500° F. with 64 grams of powdered calcium carbide. A gaseous reaction product containing acetylene was formed and removed. The product remaining in the reaction zone was a dark-colored brittle solid at room temperature and comprised a calcium salt of the alkylated phenol. 94% of the theoretical yield of calcium alkyl phenate was obtained as shown by an analysis of a sample of the reaction product freed from calcium carbide by filtration of its petroleum ether solution.

*Example 4.*—685 grams of an alkylated phenol having an apparent molecular weight of 290 were agitated for six hours at approximately 500° F. to 540° F. with 90 grams of calcium carbide. A gas containing acetylene was formed and removed. The product remaining in the reaction zone was a dark-colored brittle solid at room temperature. A yield of calcium alkyl phenate, representing 96% of that theoretically possible, was obtained.

*Example 5.*—44 grams of p-cyclohexyl phenol and 20 grams of powdered calcium carbide were heated together at 350° F. for one hour. The product was a tan-colored powder insoluble in petroleum ether, soluble in benzene, and comprising the calcium salt of p-cyclohexyl phenol.

*Example 6.*—234 grams of an alkyl cresol (molecular weight 291) and 25 grams of powdered calcium carbide were heated at 530° F. with stirring for four hours. The product obtained comprising the calcium salt of alkyl cresol was a hard brittle solid, soluble in mineral oil.

It is believed that the reactions occurring in the above examples may be represented by the following equation:



Metal carbides other than calcium carbide give the above type reaction and may be utilized. Such other compounds comprise those metal carbides which are known to react with water to yield acetylene. These metal carbides are herein termed "acetylides" and comprise the carbides of the alkali metals and the alkaline earth metals, namely, sodium, potassium, rubidium, cesium, lithium, magnesium, calcium, strontium and barium.

Additional examples of methods of preparing metal phenates useful in the compositions of this invention comprise the following:

*Example 7.*—To 217 grams of an alkyl phenol (molecular weight 290) was added 17.2 grams of sodium metal. The temperature was maintained at approximately 350° F. and the sodium metal added in small pieces while the mixture was stirred mechanically. The evolution of hydrogen was quiet and the time for completion of the reaction was about three hours. At 300° F. the product was a viscous brown liquid. Mineral lubricating oil was added at this temperature to give a 1% solution of the compound.

*Example 8.*—100 grams of an alkyl phenol (molecular weight 290) and 15 grams of aluminum wire were heated together. A crystal of iodine was added as a catalyst. The reaction continued until no further hydrogen evolution was evident. The product was dissolved in petroleum ether, filtered, and the petroleum ether evaporated on a steam bath.

*Example 9.*—500 grams of an alkyl phenol (molecular weight 290) were heated to 520 to 540° F. and a crystal of iodine was added. 30 grams of magnesium turnings were then incorporated in small increments to maintain a rapid but safe evolution of hydrogen. Before the en-

re quantity of magnesium had been added, the eaction mixture became too viscous to stir even at 600° F. This mixture was dissolved in acid treated S. A. E. 30 Western lubricating oil and topped to 480° F. at 5 mm. pressure in a still.

**Example 10.**—7.6 grams of barium hydroxide were dissolved in 7 cc. of water at 212° F. To this was added, with agitation, about 5 grams of cetyl phenol and 7 cc. of ethyl alcohol to promote solution of the cetyl phenol and facilitate reaction. The mixture was boiled for about three minutes, extracted with a hydrocarbon thinner, the extract filtered and the thinner evaporated. The product obtained was an amber, brittle semi-solid containing approximately 65% of the barium salt of cetyl phenol. The reaction product as obtained was dissolved as a 1% solution in lubricating oil and found by engine test to satisfactorily inhibit piston ring sticking.

To illustrate the preparation of calcium chloroamyl phenate and oils containing the same, the following is given:

**Example 11.**—82 grams of p-tertiary amyl phenol was dissolved in 500 cc. of 50% alcohol. Chlorine was bubbled through the solution for ten minutes, keeping the solution out of the sunlight. A heavy oil precipitated and was drawn off. The oil was dissolved in petroleum ether and washed several times with  $\text{Na}_2\text{S}_2\text{O}_3$  solution and with water. Solvent was removed on a steam bath. Analysis:

Chlorine..... per cent 21.32  
Neutralization No. .... 290

70 grams of this chloroamyl phenol was mixed with 22 grams  $\text{Ca}(\text{OH})_2$  and 1 liter of a petroleum hydrocarbon thinner. This mix was refluxed at about 220° F., the water being collected, for four hours. The petroleum hydrocarbon solution was filtered and gave 5-10 grams of an amber-colored semi-solid on removal of solvent. The residue from filtration was extracted with boiling benzene, and on removal of the benzene yielded about 45 grams of a white solid. Analysis of white solid



|          |          |      |
|----------|----------|------|
| Carbon   | per cent | 50.6 |
| Hydrogen | do       | 6.1  |
| Ash      | do       | 27.7 |

The chloroamyl phenate was dissolved in an acid refined naphthenic base oil, S. A. E. 30, and the compounded oil filtered. The compounded oil contained about 0.25% of the calcium salt and the results obtained on testing are given in the table page 3.

**Example 12.**—Magnesium soap of chloro-p-tertiaryamyl phenol was prepared by heating magnesium metal with the phenol at 350° F. in the presence of a crystal of iodine. Hydrogen was evolved and the mass became semi-solid.

**Example 13.**—Chloro-tertiaryamyl phenol (per cent chlorine—14.6), 100 grams, and aluminum wire, 7 grams, were heated together in the presence of a crystal of iodine. Unreacted phenol was distilled off and the phenate dissolved in petroleum ether. This solution was filtered and solvent removed. The product was a hard brittle solid with the following analysis:

|                  |          |       |
|------------------|----------|-------|
| Carbon           | per cent | 51.49 |
| Hydrogen         | do       | 6.76  |
| Ash              | do       | 20.2  |
| Molecular weight |          | 428   |

The proportion of metal phenates added to mineral lubricating oils may vary widely, depending upon the uses involved and the properties desired. As little as 0.1% by weight of the phenate gives measurable improvements, although from approximately 0.25 to approximately 2% phenate is preferred where the compounded oil is to be used as a crankcase lubricant for internal combustion engines. As much as 50% by weight of various of the phenates may be dissolved in mineral oil for the purpose of preparing a concentrate capable of dilution with lubricating oils and the like. Such concentrates comprise a convenient method of handling the phenates and may be used as a compounding agent for lubricants in general, as well as for other purposes.

The advantages of the compounded hydrocarbon oils of this invention are illustrated by the following test data:

| Oil                                                              | Time to stick rings |                   | Relative corrosion<br>Cd-Ag<br>bearings | Relative<br>ring slot<br>carbon | Relative<br>piston<br>cleanliness | Used oil inspections |                   |              | Remarks                                           |
|------------------------------------------------------------------|---------------------|-------------------|-----------------------------------------|---------------------------------|-----------------------------------|----------------------|-------------------|--------------|---------------------------------------------------|
|                                                                  | Hours               | Comp./min.<br>oil |                                         |                                 |                                   | Vis. @<br>100° F.    | Vis. @<br>210° F. | Neut.<br>No. |                                                   |
| Acid refined, S. A. E. 30, Western oil—No. 1.                    |                     | (*)               | 1.0                                     | Very low.                       | Poor.....                         | 906                  | 64.3              | 0.72         |                                                   |
| Oil No. 1 plus 0.96% aluminum di(cetyl phenate).                 | 90                  | 3.0               | do.....                                 | Excellent                       | Good.....                         | 1,620                | 79.7              | 5.54         | Made with aluminum metal and cetyl phenol.        |
| Oil No. 1 plus 1% barium cetyl phenate.                          | 45+                 | 1.5+              | Low.....                                | Good.....                       | Fair.....                         | 1,045                | 67.1              | 0.90         | Made by reaction with barium hydroxide.           |
| Oil No. 1 plus 1.1% calcium cetyl phenate.                       | 90+                 | 3.0+              | Very low.                               | Excellent                       | Very good                         | 1,490                | 76.7              | 3.87         | Made with calcium metal and cetyl phenol.         |
| Oil No. 1 plus 1.0% calcium cetyl phenate.                       | 165+                | 5.5+              | do.....                                 | Perfect.....                    | do.....                           | 1,915                | 86.2              | 3.96         | Check run on above.                               |
| Oil No. 1 plus .88% calcium cetyl phenate.                       | 135+                | 4.5+              | do!                                     | do.....                         | Good.....                         | 1,576                | 79.7              | 3.63         | Made from calcium carbide and cetyl phenol.       |
| Oil No. 1 plus 0.92% calcium cetyl phenate.                      | 120+                | 4.0+              | Low.....                                | Very good                       | Fair.....                         | 1,764                | 84.1              | 3.54         | Made from calcium metal and cetyl phenol.         |
| Oil No. 1 plus 0.96% calcium cetyl phenate.                      | 120                 | 4.0               | Medium <sup>1</sup>                     | do.....                         | Good.....                         | 1,480                | 57.9              | 3.45         | Cetyl phenol made by aluminum chloride method.    |
| S. A. E. 30, Western oil—No. 2 plus 0.74% calcium cetyl phenate. | 45+                 | 1.5+              | .....                                   | Fair.....                       | Poor.....                         | 1,000                | 68.7              | 1.42         | Tests on compounding agent in different oil.      |
| Oil No. 2 plus 1.22% calcium cetyl phenate.                      | 105                 | 3.5               | Very low <sup>1</sup>                   | Good.....                       | Very good                         | 1,080                | 70.9              | 1.85         |                                                   |
| Oil No. 1 plus 1% calcium di-ethyl phenate.                      | 60                  | 2.0               | do.....                                 | do.....                         | Fair.....                         | 1,250                | 72.5              | 2.06         | Made with calcium metal and di-ethyl phenol.      |
| Oil No. 1 plus 1% calcium di-ethyl phenate.                      | 60+                 | 2.0+              | High.....                               | do.....                         | do.....                           | 1,425                | 75.7              | 3.01         | Made with calcium metal and "heptyl" phenol.      |
| Oil No. 2 plus 1.55% calcium lauryl phenate.                     | 120+                | 4.0+              | Medium <sup>1</sup>                     | Excellent                       | Good.....                         | 1,107                | 72.2              | 0.81         | Made with calcium metal and lauryl phenol.        |
| Oil No. 1 plus 1% calcium p-tertiary amyl phenate.               | 45                  | 1.5               | Very low <sup>1</sup>                   | Fair.....                       | Fair.....                         | 1,180                | 69.2              | 1.87         | Made with calcium metal and tertiary amyl phenol. |
| Oil No. 1 plus 0.24% calcium mono-chloroamyl phenate.            | 30                  | 2.0               | Medium.....                             | do.....                         | Poor.....                         | 742                  | 67.6              | 3.08         |                                                   |

<sup>1</sup> Corrosion data not from engine test.

<sup>2</sup> Ratio of time required to stick rings with compounded oil as compared with uncompounded mineral oil.

In the above piston ring sticking tests, a single cylinder 2 $\frac{5}{8}$ " bore, 2 $\frac{1}{2}$ " stroke, Lauson gasoline engine was operated under extremely severe conditions for the purpose of developing fully piston ring sticking and piston gumming tendencies under circumstances simulating severe operating conditions encountered in the field. Operation of the motor during tests was continuous at 1600 R. P. M. except for periodic shut-downs at fifteen hour intervals for inspection; the jacket temperature was maintained at 345° F. and sump oil temperature at 220° F. The corrosion data given, except where noted otherwise, were determined by measuring the loss of weight of metal from the bearings during runs with this type of engine under the above severe conditions.

The metal phenates of this invention may be added to mineral oils containing other compounding ingredients, such as pour point depressors, oiliness agents, extreme pressure addition agents, corrosion inhibitors, blooming agents, compounds for enhancing the viscosity index of the hydrocarbon oil, etc. The invention in its broader aspects embraces mineral hydrocarbon oils containing the metal phenates in which thickening agents and/or metal soaps may be present either in grease-forming proportions or in amounts insufficient to form greases, as in the case of mineral castor machine oils.

In the foregoing disclosure, calcium salts of chlorinated phenols and magnesium salts of chlorinated phenols have been referred to and described merely to illustrate the general group of polyvalent metal salts of halogenated phenols. The other metal phenates herein disclosed may be halogenated and utilized according to the teachings of the present invention. In the halogenated compounds the chlorine or halogen atom may be present either in the aryl portion of the molecule, that is, in the benzene ring to which the metal is attached through an oxygen atom, or the halogen atom may be contained in the substituent of hydrocarbon structure attached to said benzene ring. Further, the halogen atom may be substituted in both places, that is, directly in the ring and in the substituent of hydrocarbon structure.

While the character of the invention has been described in detail and numerous examples of the preparation and application of the composition given, this has been done by way of illustration only and with the intention that no limitation should be imposed on the invention thereby. It will be apparent to those skilled in the art that numerous modifications and variations of the illustrative examples may be effected in the practice of the invention which is of the scope of the claims appended hereto.

We claim:

1. A composition of matter comprising a hy-

drocarbon oil and more than approximately 0.1% by weight based on the oil of a metal phenate containing a halogenated phenolic radical having more than ten carbon atoms.

2. A composition as defined in claim 1 in which the phenate is an alkaline earth metal phenate.

3. A composition as defined in claim 1 in which the phenate is a calcium phenate.

4. A lubricating composition comprising a hydrocarbon oil and more than approximately 0.1% by weight based on the oil of a metal phenate containing a mononuclear phenolic radical, said phenolic radical containing chlorine and an alkyl group having more than four carbon atoms.

5. A lubricating composition comprising a hydrocarbon oil and more than approximately 0.1% by weight based on the oil of a metal phenate containing a mononuclear phenolic radical, said phenolic radical containing a halogenated alkyl group having more than four carbon atoms.

6. A lubricating composition comprising a hydrocarbon oil and more than approximately 0.1% by weight based on the oil of an alkaline earth metal phenate containing a mononuclear phenolic radical, said phenolic radical containing a halogenated alkyl group having more than four carbon atoms.

7. A lubricating composition comprising a hydrocarbon oil and more than approximately 0.1% by weight based on the oil of a calcium phenate containing a mononuclear phenolic radical, said phenolic radical containing a halogenated alkyl group having more than four carbon atoms.

8. A lubricating composition comprising a hydrocarbon oil and more than approximately 0.1% by weight based on the oil of a metal phenate containing a phenolic radical having more than ten carbon atoms and halogenated in the aryl portion thereof.

9. A lubricating composition comprising a hydrocarbon oil and more than approximately 0.1% by weight based on the oil of an alkaline earth metal phenate containing a phenolic radical having more than ten carbon atoms and halogenated in the aryl portion thereof.

10. A lubricating composition comprising a hydrocarbon oil and more than approximately 0.1% by weight based on the oil of a calcium phenate containing a phenolic radical having more than ten carbon atoms and halogenated in the aryl portion thereof.

11. A compounded lubricant comprising a hydrocarbon oil and from approximately 0.1% to approximately 2% by weight based on the oil of a polyvalent metal phenate containing a halogenated phenolic radical having more than ten carbon atoms.

ELMSLIE W. GARDINER,  
GEORGE H. DENISON, JR.